# EUROPEAN PATENT SPECIFICATION

(11) **EP 0 148 268 B1**
(45) Date of publication and mention of the grant of the patent: **19.08.1987**
(21) Application number: 83901615.1
(22) Date of filing: 18.05.1983
(51) Int. Cl.: C25D 5/26, C25D 3/22

(54) **PROCESS FOR PRODUCING STEEL STRIP ELECTROPLATED WITH ZINC ON BOTH SIDES IN CHLORIDE BATH**
VERFAHREN ZUM ERZEUGEN VON BEIDSEITIG ELEKTROZINKPLATTIERTEN STAHLBÄNDERN IN EINEM CHLORIDBAD
PROCEDE DE PRODUCTION D'UNE BANDE EN ACIER ZINGUEE DES DEUX COTES PAR UN PROCEDE GALVANIQUE DANS UN BAIN DE CHLORURE

(43) Date of publication of application: 17.07.1985
(73) Proprietor: KAWASAKI STEEL CORPORATION, Chuo-Ku, Kobe-City Hyogo 651 (JP)
(72) Inventor: MATSUDA, Akira, Chiba 281 (JP); KIMURA, Hajime, Kurashiki City, Okayama 712 (JP)
(74) Representative: Overbury, Richard Douglas
(86) International application number: JP8300147
(87) International publication number: WO8404548

## Description

This invention relates to a method of producing a both-side electrogalvanized steel strip in a chloride bath which is able to form beautiful and glossy plated surfaces by profitable improvement of zinc coating coverage in the electrogalvanizing with the chloride bath.

As a plating system in an electrogalvanizing line, there are two systems, one of which being a simultaneous both-side plating system wherein both sides of steel strip are simultaneously electrogalvanized, and the other of which being a both-side separate plating system composed of two-stage plating wherein one side of steel strip is electrogalvanized in a first plating stage and thereafter the opposed side of steel strip is electrogalvanized in a second plating stage.

The both-side separate plating system has some merits that the changeover between both-side coating and one-side coating can be achieved by merely turning over the passing direction of the steel strip to be coated, and the replacement of used electrode with new electrode can be performed simply and hence the workability is excellent.

As the both-side separate plating system, there are a horizontal type as shown in Fig. 1, and a radial type as shown in Fig. 2. In any case, a wetting tank 3 is arranged between a first plating cell 1 and a second plating cell 2. A steel strip 4 is passed through the first and second plating cells 1, 2 by means of conductor rolls 5, during which it is subjected to a galvanizing with an electrolyte 7 through an anode 6 arranged opposite to the steel strip 4.

When the steel strip 4 moves from the first plating cell 1 to the second plating cell 2, it is wetted with a wetting solution 8 in the wetting tank 3. This wetting treatment is carried out in order to introduce the steel strip 4 into the second plating cell 2 at a uniformly wetted condition of the non-plated surface, because when the non-plated surface of the steel strip 4 to be introduced into the second plating cell 2 is completely dry or is locally adhered with the electrolyte, it is apt to produce uneven plating by the second plating treatment.

Heretofore, a sulfate bath consisting essentially of zinc sulfate has mainly been used as an acidic electrolyte for the electrogalvanizing. Lately, a chloride bath becomes frequently used instead of the sulfate bath because of the following merits as compared with the sulfate bath:
(1) Since the electric conductivity is high, the required voltage can be reduced; and
(2) Since the acceptable current density is high, the high-speed plating is easy.

Incidentally, when the sulfate bath consisting mainly of zinc sulfate is used as the electrolyte, no care must be particularly taken on the wetting solution in the wetting tank 3. That is, good both-side galvanized steel strip can be obtained by using the electrolyte in itself as the wetting solution.

However, when the chloride bath consisting mainly of zinc chloride is used as the electrolyte, if such an electrolyte in itself is used as the wetting solution in the wetting tank 3, it is confirmed that the zinc coating coverage extremely lowers in a surface to be plated in the second plating cell 2.

The invention is to provide a method of producing a both-side electrogalvanized steel strip in a chloride bath which advantageously solves the aforementioned problems of the prior art in the both-side separate plating system by adding a special means to the wetting treatment prior to the second plating treatment.

The essential feature of the invention is as follows.

That is, the invention lies in a method of producing a both-side electrogalvanized steel strip in a chloride bath by plating one side of the steel strip in a first plating cell, wetting the thus one-side plated steel strip in a wetting tank, and then plating the other non-plated side of the steel strip in a second plating cell, characterized in that the concentration of zinc in the chloride wetting solution of the wetting tank is 0.1 to 50 g/I.

The invention will be described concretely based on the following experimental result.

A cold-rolled steel strip having a thickness of 0.8 mm was degreased, pickled, and then subjected on both sides to an electrogalvanizing at each coating amount of 10 g/m² under the following same plating conditions by varying only the concentration of zinc in the wetting liquid as shown in the following Table 1.

The zinc coating coverage was observed with respect to the plated surface of each of the steel strips by means of a scanning type electron microscope, and the glossiness of the plated surface (JIS Z8741) was measured by means of a glossmeter. Further, the test specimen was subjected to a humidity cabinet test, and a ratio of red rust produced after 3 days was examined. The thus obtained results are also shown in Table 1.

As apparent from Table 1, all of the bottom surfaces coated in the first plating cell had the zinc coating coverage of 100% and were good in the glossiness and the corrosion resistance according to the humidity cabinet test. In the top surfaces coated in the second plating cell, however, the zinc coating coverage was changed in accordance with the concentration of zinc in the wetting solution. That is, when the zinc concentration is exceeds 50 g/I, the zinc coating coverage rapidly lowers to leave uncoated portions and hence the corrosion resistance and glossiness are deteriorated, while when it is less than 0.1 g/I, the glossiness lowers.

According to the invention, therefore, the concentration of zinc in the wetting solution to be used in the chloride wetting tank is limited to a range of 0.1 to 50 g/I.

Although the reason why the zinc concentration in the wetting tank has an influence on the zinc coating coverage is not clear, it is anticipated that when the steel strip is previously wetted with a solution having high zinc concentration, zinc is adsorbed on the surface of the strip, and when the wetted strip is subjected to subsequent plating, the selective electrodeposition is promoted because crystals grow about the adsorbed zinc. Thus, it is considered that the crystal growth is preferential rather than the nuclear formation so that the strip surface can not uniformly be coated with zinc and consequently the zinc coating coverage is deteriorated. On the other hand, when the zinc concentration is low, the adsorption of zinc is small, which is considered to have no influence on the subsequent plating.

The composition other than zinc in the wetting solution is not particularly critical, but it is desirable to use the same composition system as in the electrolyte in view of the introduction of the wetted strip into the subsequent plating cell.

The temperature of the wetting liquid is not critical, but it is practically 20-50°C. And also, pH of the wetting solution does not substantially affect the zinc coating coverage and is not restricted, but it is preferably about 3-6.

The wetting treatment may be carried out in the usual manner such as dipping method, spraying method or the like.

The chloride bath to be used in the invention consists mainly of zinc chloride and, if necessary, contains as a conductive assistant a proper amount of at least one substance selected from ammonium chloride, potassium chloride, sodium chloride, aluminum chloride, barium chloride, calcium chloride and magnesium chloride. In general, the concentration of zinc chloride is within a practical range of 100-300 g/l, and the concentration of chloride as the conductive assistant is 100-450 g/l. Furthermore, other additives such as gloss agent, pH buffer and the like may be added.

As mentioned above, according to the invention, the both-side electrogalvanized steel strip having improved zinc coating coverage, glossiness and corrosion resistance can be produced from the chloride plating cells by adjusting the concentration of zinc in the chloride wetting solution of the wetting tank to a range of 0.1-50 g/I.

The invention will now be described in detail with reference to the accompanying drawings, wherein:
Fig. 1 is a diagrammatical view of a horizontal-type both-side electrogalvanizing line; and
Fig. 2 is a diagrammatical view of a radial-type both-side electrogalvanizing line.

A steel strip was subjected to a both-side electrogalvanizing at a coating weight per one side of 20 g/m² under the following plating conditions using a combination of a chloride plating bath and a wetting solution each having a composition shown in the following Table 2 and then examined with respect to the zinc coating coverage and glossiness to obtain results as shown in Table 2.

### Plating conditions

As apparent from the results of Table 2, the plated steel strips having good zinc coating coverage and glossiness are obtained in the cloride bath having the composition according to the invention. In Run Nos. 8 and 9 wherein the zinc concentration of the wetting solution is outside the range defined in the invention, the glossiness or zinc coating degree of the plated surface is poor.

As apparent from the above examples, according to the invention, the both-side electrogalvanized steel strip having the improved zinc coating coverage and glossiness can be produced in the chloride bath by limiting the zinc concentration of the wetting solution to 0.1-50 g/I.

In the production of both-side galvanized steel strips according to the invention, very glossy and beautiful plated surface can be obtained even when being subjected to high-speed electrogaLvanizing using a chloride bath, so that mass production can easily be realized in industrial scale and also the reduction of the cost is achieved.

## Claims

A method of producing a both-side electro-galvanized steel strip in a chloride bath by plating one side of the steel strip in a first plating cell, wetting the thus one-side plated steel strip in a wetting tank, and then plating the other non-plated side of the steel strip in a second plating cell, characterized in that the concentration of zinc in the chloride wetting solution of the wetting tank is 0.1 to 50 g/I.

## Patentansprüche

Verfahren zur Erzeugung eines beidseitig elektrogalvanisch behandelten Stahlbands in einem Chloridbad, wobei zunächst die eine Seite des Stahlbands in einer ersten Platierzelle platiert, dann das so einseitig platierte Stahlband in einem Benetzungsbehälter befeuchtet und schließlich die andere, noch nicht platierte Seite des Stahlbands in einer zweiten Platierzelle platiert wird, dadurch gekennzeichnet, daß die Zinkkonzentration der im Benetzungsbehälter vorhandenen Chloridbefeuchtungslösung 0.1-50 g/I beträgt.

## Revendications

Une méthode de fabrication d'une feuille d'acier électro-galvanisée sur les deux faces dans un bain de chlorure par placage d'une face de la feuille d'acier dans une première cuve de placage, mouillage de la feuille l'acier ainsi plaguée sur une face dans un bac de mouillage, et ensuite placage de l'autre face non plaquée de la feuille d'acier dans une deuxième cuve de placage, la dite méthode étant caractérisée en ce que le concentration en zinc dans la solution de mouillage au chlorure du bac de mouillage est de 0,1 à 50 g/1.
